

## UNITED STATES PATENT OFFICE

2,155,894

## METHOD OF PRODUCING COLORED PICTURES AND SOUND FILMS

Béla Gáspár, Brussels, Belgium

No Drawing. Application April 5, 1938, Serial No. 200,218. In Germany June 15, 1933

3 Claims. (Cl. 95—2)

This invention relates to a method of making colored movie films having a black and white sound record, more particularly a sound record which comprises a metallic deposit image, and is a continuation-in-part of my prior application Serial No. 730,259, filed June 12, 1934.

Such a black and white sound record is preferable in many respects to a sound record having a sound image in some particular color because it is very difficult to reproduce the blackening curve without distortion, by a colored sound record. This is especially true in connection with so-called variable intensity recording. Furthermore, a sound image in a particular color requires a photoelectric cell sensitive to a particular colored light in order to reproduce it and a black and white record can be reproduced by any photoelectric cell. However, known processes for combining a colored picture image and a black and white sound record present the difficulty of being unusually complicated because of various factors, such as necessity for local treatment of the sound track, covering the sound track with a resist or a protective coating during certain steps in the process of making the colored picture portion, etc.

It is therefore an object of this invention to provide an improved method of easily and cheaply making a colored film having a black and white sound record.

I have discovered that most of the processes utilized in the production of colored film involving the intermediate production of a metallic deposit image include a treatment which weakens and hence deteriorates the quality of the metallic deposit image. In those processes where the metallic deposit image is ultimately removed, such deterioration causes no difficulty. On the other hand, when the film carries a metallic deposit sound record which it is desired to preserve, and both the picture and sound portion of the film are given common treatment, this weakening of the sound record results in a decrease in the quality of sound reproduction.

It is therefore a further object of my invention to obviate this difficulty by an improved method of making a colored film having a metallic deposit sound record.

In accordance with my invention I make the metallic deposit image in the sound track of excessive density prior to any treatment which may cause a weakening of the record. As a result, the excess density compensates for the subsequent weakening of the image and a resultant sound record is produced which possesses the de-

sired normal density. The excessive density may be obtained by excessive exposure or by excessive development of the sound image, or by both methods combined. One may thereby obtain a sound record which, despite subsequent weakening arising from later treatment of the film, is still adequate to permit proper reproduction of sound.

The black and white sound record may be produced as a pure black silver image, or the same may be colored, or, if previously colored, it may be allowed to remain in colors.

The colored film may be produced as desired. Thus, for example, there may be used the well-known mordanting process, in which the silver image is first converted into a mordant, such as silver thiocyanate or silver ferrocyanide, whereupon coloring is performed with a suitable dyestuff. In this case after the coloring of the silver salts which act as a mordant for the dyestuff, the sound portion of the film will be treated with developer which reduces the silver salt to silver, and a silver sound record comprising both black silver and dyestuff will be obtained. If the sound track is treated with a sodium hydro-sulphite solution, a pure black silver sound image will be obtained adjacent to the colored image portion.

The process according to the invention is particularly suitable in conjunction with the processes which I have described in my prior Patent No. 1,985,344, December 25, 1934, and my prior Patent No. 2,025,658, December 24, 1935.

According to the Patent No. 1,985,344, there is employed a film material comprising three differently colored and differently sensitized layers poured one on to the other and composed, for example, as follows:

| Layer | Color      | Sensitization of silver halide layer | 40 |
|-------|------------|--------------------------------------|----|
| III   | Magenta    | Blue.                                |    |
| II    | Yellow     | Red.                                 | 45 |
| I     | Blue-green | Infra red.                           |    |

The picture portion is copied into the single layers in the known fashion by the use of master positives, which correspond to the negative color selection pictures. For copying the sound record, layers III and II, for example, are exposed diffusely, and layer I is exposed behind a sound negative with infra-red light, copying being performed to such an extent that the layer 50 55

I is over exposed whereby the density of the sound image when developed will be greater than the requisite density in the finished film. Actually this initial density is increased by approximately 40%.

Instead of over exposing layer I to obtain a sound image of greater than normal density, I may give a normal exposure at the time of printing the sound record and obtain the abnormal density by over-developing the sound record portion of the film.

The developed silver image comprising the picture and sound portions may be treated in accordance with Patent No. 2,020,775, November 12, 1935, with an acid thiocarbamide solution, which may have, for example, the following composition:

|                  | Parts |
|------------------|-------|
| Water            | 100   |
| 20 Thiocarbamide | 5     |
| Citric acid      | 2     |

the dyestuff then being destroyed at the points of the silver deposit and maintained at the points which are free of silver. Finally, the silver deposit in the picture portion of the film is dissolved out with the aid of a suitable silver solvent, such as Farmer's reducer.

The film now possesses in the picture portion a pure dyestuff image, and in the sound portion a metallic silver sound record on a blue-green background. If it is desired to have a pure silver image in the sound area of the film, the sound record is treated with a dyestuff destroying agent for example with sodium hydrosulphite, titanium trichloride, tin chloride, etc., possibly with the addition of accelerating agents such as acids or indulin scarlet. The degree of decolorization may be made to vary. If desired, the color in the sound area of the film may be reduced or destroyed only to such extent as may be necessary to permit of a proper reproduction. These diffuse dyestuff destroying agents for treatment of the sound record may be used at any suitable time during the process of converting the picture portion of the metallic deposit film into a color film. Thus, for example, following the dyeing process or after the dye destroying operation performed to produce the colored image.

In those cases in which a film is colored with a number of colors resulting in subtractive black, as is the case in the above example, it will be found sufficient to remove from the sound record merely one of the colors, for instance the color absorbing the rays which are most effective on the reproducing cell.

Instead of employing layers to which the dyestuff is previously applied, i. e., predyed layers, these layers may also be colored after exposure. For example, one may use dyestuff-forming substances, such as leuco-esters or amines. Azo dyestuffs may also be produced in the film in the same fashion.

Processes of this nature are described, for example, in my Patent No. 2,071,688, February 23, 1937. The dyestuff is formed diffusely, and then destroyed locally. Alternatively the dyestuff-forming substance may be destroyed locally and the remaining substance then converted into a dyestuff.

While I have described my improved process by reference to a particular adaptation, it will be

understood that this is only exemplary. My improved method is applicable to all known methods for the production of colored picture and sound films, even though the film includes one or more layers on one or on both sides of the backing or support, and I intend to include all modifications which come within the scope of my invention, as set forth in the appended claims.

What I claim as new and desire to secure by Letters Patent is:

1. A method of producing combined colored picture and sound films including a picture portion and a sound track wherein the sound image comprises a metallic deposit, which comprises forming a metallic image in the picture portion of said film of normal density and forming a metallic sound image in the sound track of greater density than that required in the finished film for adequate sound reproduction, and subsequently treating the whole film to convert the metallic image in said picture portion to a colored image by means of an agent which decreases the density of said metallic images, said excess density of said metallic sound image being so regulated as to compensate for the decrease in density of said metallic sound image during treatment of said film to convert the metallic image in the picture portion to a color image and to thereby form a normal density metallic sound image.

2. A method of producing combined colored picture and sound films including a picture portion and a sound track wherein the sound image comprises a metallic deposit, which comprises forming a metallic image in the picture portion of said film by normal exposure and forming a metallic sound image in the sound track of greater density than that required in the finished film for adequate sound reproduction, by over-exposure, and subsequently treating the whole film to convert the metallic image in said picture portion to a colored image by means of an agent which decreases the density of said metallic images, said over-exposure in said sound track being so regulated as to increase the density of said metallic sound image sufficiently to compensate for the decrease in density of said metallic sound image during treatment of said film to convert the metallic image in the picture portion to a color image and to thereby form a normal density metallic sound image.

3. A method of producing combined colored picture and sound films including a picture portion and a sound track wherein the sound image comprises a metallic deposit, which comprises forming a metallic image in the picture portion of said film by normal development and forming a metallic sound image in the sound track of greater density than that required in the finished film for adequate sound reproduction by over-development, and subsequently treating the whole film to convert the metallic image in said picture portion to a colored image by means of an agent which decreases the density of said metallic images, said over-development in said sound track being so regulated as to increase the density of said metallic sound image sufficiently to compensate for the decrease in density of said metallic sound image during treatment of said film to convert the metallic image in the picture portion to a color image and to thereby form a normal density metallic sound image.

BÉLA GÁSPÁR.